

## UNITED STATES PATENT OFFICE

JOHN E. WOODWARD, OF BROOKLYN, NEW YORK, ASSIGNOR TO MESSRS. KASTENHUBER & LEHRFELD, OF NEW YORK, N. Y., A PARTNERSHIP CONSISTING OF CHARLES F. KASTENHUBER, WILLIAM F. LEHRFELD, AND HUGO R. LEHRFELD

## PEN-POINT ALLOY

No Drawing.

Application filed December 19, 1927. Serial No. 241,278.

This invention relates to alloys and more particularly to an alloy for a pen point though it is noted that the invention is not limited to pen points.

5 One of the main objects of my invention is to provide an economical osmium alloy for use as a pen point.

Another object of my invention is to provide an economical osmium alloy that is 10 tough, durable and which will take a high polish.

Another object of my invention is to provide a base alloy of nickel and tungsten that can be shipped to manufacturers of pen points 15 who can then alloy the base alloy with osmium in the way I shall describe later.

Still another object of my invention is to provide an alloy of osmium with tungsten and nickel which will be tough, acid resisting, 20 have a durable wearing surface, take a high polish and be economical to produce.

And still another object of my invention is to provide a pen point made of an alloy osmium, tungsten, nickel and if desired platinum, which will take a high polish and have 25 durable wearing surface, and be tough, fusible with great difficulty, be readily capable of soldering or freezing to a gold nib, and yet be economical to produce.

30 Still other objects of my invention will appear as the description proceeds; and while herein details of the invention are described and claimed, the invention is not limited to these.

35 It is a well known fact in the art of making alloy pen points that osmium is a desirable hardening constituent in pen point alloys. It has been found that the hardness of such alloys increases in proportion to the amount 40 of osmium present therein. Osmium in the pure state is incapable of use in the above respect. It is too brittle and friable. After fusion, and upon cracking or crushing, a pure osmium button (or even the native osmiridium button) powders readily. This results 45 in a very serious loss since these metals are rare and precious, and much of the powder gets lost.

It is therefore necessary to add a so-called 50 toughening agent or metal to osmium in

order to give it the strength required for practicable and economical commercial use. Toughening metals that have been added heretofore are either of two kinds:—

(a) Metals of the platinum group 55

(b) Base metals such as nickel, cobalt, etc., or any element or combination of elements which can impart the required strength and toughness to the osmium metal.

The objection to the use of the platinum 60 metals other than osmium by themselves is that they are comparatively soft, and therefore reduce the hardness of the resultant alloy with osmium. The objection to the use of the base metals alone is that they do not form 65 true solutions or alloys with osmium. Thus upon cooling, segregation takes place and the resultant alloy is not of a homogeneous texture. Consequently a high polished surface 70 of uniform appearance cannot be procured.

Now I have discovered an alloy and a method of producing the same which will overcome all the above obstacles. I have discovered a method of introducing a toughening alloy into the osmium metal whereby a perfectly homogeneous alloy is produced and what is most important very little of the hardness of the osmium is lost. 75

I have found that altho the metal tungsten when melted with osmium does not form a 80 true solution, yet if the tungsten be first dissolved in nickel, an alloy results which will form with osmium a true solution and alloy, that will impart to osmium the desired toughness, homogeneous texture and durable 85 wearing surface.

In fact a dual advantage is accomplished by my newly discovered process. It will be observed that I substitute a larger percentage 90 of base metals for rare or semi-rare metals heretofore utilized in this art, and yet I am able to equal any of the characteristics of the expensive rare metal alloys.

It will further be noted that I provide a base alloy that can be shipped as a sort of 95 intermediate product to pen manufacturers, there to be alloyed with osmium to produce my novel alloy.

My process consists then in heating nickel (M. P. 1484° C.) and adding thereto tung- 100

sten (M. P. 3500° C.) as the nickel fuses. The proportions for a given batch of base alloy, as I prefer to call this alloy of nickel and tungsten, is 75% of tungsten and 25% of nickel. At about 1900° C. it was found that a true solution took place. That is to say the base alloy melts at about 1900° C. It exhibits a uniform texture or polishing thus showing that it is free from segregation and is a homogeneous alloy.

I then may chill the tungsten-nickel solution, or I may add the osmium metal. I use 80% of osmium (M. P. 2400° C.) and 20% of the base alloy for a given batch of my final alloy. I find that at 2400° C.—a true solution of osmium, tungsten and nickel results. The resulting alloy at this point, upon chilling, has a uniform homogeneous texture and takes a very high polish.

I can use other metals of the nickel group such as cobalt. I can likewise use other metals of the tungsten group as molybdenum. Altho I have given 80% of osmium as a preferable proportion of that metal, I have found that I can use from 70-85% of osmium and from 30-15% of my base alloy and still get good results.

To utilize my alloy a button of it is stamped, cracked or crushed to obtain pieces for freezing on to gold nibs and finishing as pen points and similar wearing surfaces. I find that my alloy does not powder when crushed. I get an alloy which hangs together when crushed and does not powder. I get particles suitable for polishing and working. I, then, greatly reduce the loss due to powdering and yet use inexpensive materials. The texture is uniform and homogeneous and the surface of the pen point takes on a very high polish thus resulting in a smoothly writing point.

I desire to point out that platinum (M. P. 1745° C.) may be added to increase the toughness. If so desired then it is added before the osmium is dissolved in the tungsten-nickel alloy in the proportion of 10%. Then 80% of osmium is added. The base alloy would be present to the amount of 10%.

The characteristics of this alloy with added platinum are still preserved if the ranges of percentages of the ingredients of the final alloy do not exceed the following:

5-15% of tungsten;  
1-5% of nickel;  
5-15% of platinum; and  
70-85% of osmium.

The osmium alloy need not be formed immediately after the nickel-tungsten alloy. After the base alloy has been formed, I can chill it and ship it to pen manufacturers. In other words I thus provide a basic material or intermediate as a new composition of matter. Altho, this material may not be of much use itself, yet upon being processed with osmium in the proportions described above—

a finished product is obtained that can then be used in the manner I have outlined above.

So also I am not limiting myself to the temperatures mentioned above. I include within the scope of the appended claims any range of temperatures which will produce my novel alloy.

What I claim is:—

1. An alloy comprising 80% of osmium; 10% of platinum; and 10% of a base alloy comprising 75 parts of tungsten to 25 parts of nickel.

2. An alloy comprising 70-85% of osmium; 10% of platinum; and 10% of a base alloy comprising 75 parts of a metal of the tungsten group and 25 parts of a metal of the nickel group.

3. An alloy comprising 70-85% of osmium; 10% of platinum; and 5 to 20% of a base alloy comprising 75 parts of tungsten to 25 parts of nickel.

4. An alloy comprising 70-85% of osmium; 5-15% of a metal of the platinum group other than osmium; and 5-20% of a base alloy comprising 65-85 parts of a metal of the tungsten group to 15-35 parts of a metal of the nickel group.

5. An alloy comprising 5-15% of a metal of the tungsten group; 1 to 5% of a metal of the nickel group; 5-15% of platinum; and 70-85% of osmium.

Signed at New York in the county of New York and State of New York this 17th day of December, A. D. 1927.

JOHN E. WOODWARD.

100

105

110

115

120

125

130